

## UNITED STATES PATENT OFFICE.

EUGEN VADERS, OF HEDDERNHEIM, NEAR FRANKFORT-ON-THE-MAIN, GERMANY,  
ASSIGNOR TO HEDDERNHEIMER KUPFERWERK UND SUEDDEUTSCHE KABEL-  
WERKE, AKTIENGESELLSCHAFT, OF FRANKFORT-ON-THE-MAIN, GERMANY, A COR-  
PORATION OF GERMANY.

## BEARING METAL.

No Drawing.

Application filed December 1, 1923. Serial No. 678,050.

*To all whom it may concern:*

Be it known that I, EUGEN VADERS, citizen of the German Republic, residing at Heddernheim, near Frankfort-on-the-Main, 5 Germany, have invented certain new and useful Improvements in Bearing Metal, of which the following is a specification.

This invention relates to the manufacture of bearings by the press method. The manufacture of articles from suitable brass alloys by pressing is well known. While formerly each piece had to be separately formed and cast, a single steel form is now sufficient to press a large number of articles and the 10 cost of production is reduced in proportion. Pressed articles, in addition, are generally free of defects and need little machining, while castings, as a rule, have many imperfections as is well known.

20 The object of my invention is the manufacture of bearings by pressing. Hitherto bearings and bushes could not be manufactured by this method as the known plastic alloys were not anti-frictional. To produce 25 anti-friction metal, theory requires, that in the soft matrix of a metal must be embedded hard constituents, formed by a compound or by mixed crystals, which hold the pressure of the shaft and improve the distribution of the oil. In accordance with my invention I have found, that by addition of 30 certain metals, plastic brass alloys may be obtained, having the above structure and in consequence all those qualities that are 35 necessary for bearing-metals. I have found that silicon is absolutely essential as a constituent of such hard compounds or mixed crystals to be added to ordinary press-brass to make it suitable as a bearing metal. The 40 addition of silicon to brass is old, in itself, but as appears from the literature, silicon has a detrimental effect upon the properties of brass. According to the present invention, concurrently with silicon there are 45 added other metal constituents which not only counteract or eliminate these detrimental effects of the silicon, but even produce a substantial improvement in the mechanical qualities of the metal, aside 50 entirely from the surprising anti-frictional

character thereof. Of the metals to be added together with silicon, manganese and iron have been found to be particularly suitable for the production of the hard compounds and mixed crystals within the brass 55 matrix. Addition of manganese or iron or both to brass is not new, in itself, but within the scope of my invention it is absolutely essential that at least one of them must be present, together with silicon, and it is only 60 by such concurrent use of one of the two metals and silicon that such hard compounds or mixed crystals can be produced in the brass, making the resulting alloy suitable 65 as a bearing material.

Aside from the production of hard compounds and mixed crystals in the press brass as described, it is also highly desirable within the general object thereof to impart to matrices of copper and zinc, or copper, zinc 70 and lead, as the case may be, a harder and more uniform texture. To this end an addition of aluminum has proved very beneficial.

As an example of an alloy particularly 75 suitable for the manufacture of bearings by the press method, may serve the following composition:

58% of copper, 36-37% of zinc, 0.6-1.5% of silicon, 2-2.5% of manganese, 1.5-2% of 80 aluminum showed:

1. Tensile strength: 41-44 tons p. sq. inch.

2. Elongation: 18.4% (2", diameter  $\frac{3}{8}$ ").

Up to a load of 32 tons p. sq. inch and a rapidity of sliding of 2.7 m/sec (8' 11" / sec) the new alloy was even better than phosphor bronze, which could be judged from the lower temperature of bearings running under the same conditions. In comparison with phosphor bronze these temperatures were about 5° C. lower, in comparison with ordinary red-brass, however, the difference was about 20-30° C.

A cast bearing of the above alloy had:

Tensile strength: 32-25 tons p. sq. inch. 95

Elongation: 4-5% (2", diameter  $\frac{3}{16}$ ").

A red brass bearing of the best sort, however, has only:

Tensile strength: 16-19 tons p. sq. inch.

Elongation: 3-4% (2", diameter  $\frac{3}{16}$ "). 100

Consequently, the alloys in accordance with the above invention are also appropriate for cast bearings.

What I claim is:

- 5 1. A brass alloy containing .6-1.5% of silicon and manganese in amount sufficient to neutralize the detrimental effects of the silicon.
- 10 2. A brass alloy containing .6-1.5% of silicon and an amount of manganese up to about 4% in amount sufficient to neutralize the detrimental effects of the silicon.
- 15 3. A brass alloy containing .6-1.5% of silicon and iron in amount sufficient to neutralize the detrimental effects of silicon.
- 20 4. A brass alloy containing .6-1.5% of silicon and an amount of iron up to about 4% in amount sufficient to neutralize the detrimental effects of the silicon.
- 25 5. A brass alloy containing .6-1.5% of silicon, an amount of manganese up to about 4% sufficient to neutralize the detrimental effects of the silicon, and an amount of aluminum up to about 2% sufficient to harden and homogenize the structure of the alloy.
- 30 6. A brass alloy containing .6-1.5% of silicon, an amount of iron up to about 4% sufficient to neutralize the detrimental effects of the silicon.

effects of the silicon and an amount of aluminum up to about 2% sufficient to harden and homogenize the structure of the alloy.

7. A bearing metal containing approximately 94% of brass matrix, .6-1.5% of silicon, an amount of manganese up to about 4% sufficient to neutralize the detrimental effects of the silicon, and an amount of aluminum up to about 2% sufficient to harden and homogenize the structure of the alloy.

8. A bearing metal containing approximately 94% of brass matrix, .6-1.5% of silicon, an amount of iron up to about 4% sufficient to neutralize the detrimental effects of the silicon, and an amount of aluminum up to about 2% sufficient to harden and homogenize the structure of the alloy.

9. A bearing metal containing about 58% of copper, about 36% of zinc, 2-4% of manganese, about 2% of aluminum and .6-1.5% of silicon.

10. A bearing metal containing 58% of copper, about 36% of zinc, 2-4% of iron, about 2% of aluminum and .6-1.5% of silicon.

In testimony whereof I affix my signature.

EUGEN VADERS.